

## UNITED STATES PATENT OFFICE

2,158,050

## MOTOR FUEL

Euphime V. Bereslavsky, New York, N. Y.

No Drawing. Application March 4, 1937,  
Serial No. 128,929

8 Claims. (Cl. 44—9)

This invention relates to motor fuels, and more particularly to motor fuels having a low temperature of ignition, which are adapted for solid injection engines of the Diesel type.

5 This application constitutes a continuation in part of my application Serial Number 49,027 filed November 9, 1935, for Motor fuels.

A number of truck and bus manufacturers are now offering Diesel engines as a standard or optional equipment and railroads and aeroplane manufacturers are making some use of Diesel engines for commercial transportation. The main advantages of Diesel type or compression ignition engines are greater fuel economy and smaller 10 fire risk. They also have a high thermal efficiency, simplicity of operation and construction and the elimination of carburetors and magneto.

15 The high speed Diesel type engine is finding great favor and the high speed engine operates more efficiently and effectively with a motor fuel having a high cetane number. On the other hand most hydrocarbon products which are suitable for fuel with the Diesel type engines have a 20 low cetane number and it is desirable to change the characteristics of the fuel in order to raise the cetane number. One of the important fuel characteristics attendant a high cetane number is a prompt ignition accompanied by a high rate 25 of flame propagation. Another characteristic is a low temperature of ignition. The lower are the temperatures at which compression-ignition fuels ignite the lower may be the compression ratio of the engine burning the fuel and the more 30 easily may the engine be started.

35 One important object of the present invention is to provide an accelerator by which the burning characteristics of a compression-ignition fuel may be effectively changed to increase its cetane 40 value.

Another object of the invention is to provide an improving agent or accelerator for changing the burning characteristics of the Diesel type motor fuels by which the cetane value of the 45 fuel may be increased in substantially a direct proportion as the amount of accelerator used with the motor fuel.

Some motor fuels, particularly cracked petroleum distillates, and distillates having a high 50 percentage of unsaturated hydrocarbons have

a slow rate of flame propagation and are quite difficult to ignite. Accordingly such fuels have not been satisfactory for use in Diesel engines.

Accordingly another object of the invention is to provide a chemical compound for treating hydrocarbon distillates, particularly petroleum distillates, which have a slow rate of flame propagation and a comparatively high temperature of ignition whereby the burning characteristics of such fuels may be changed to lower the ignition 5 temperature and increase the rate of flame propagation and the cetane value of the fuel in order to improve combustion characteristics of fuel in compression ignition engines.

It is well known that the ignition quality of 15 a motor fuel is dependent upon the chemical structure of the hydrocarbons in the fuel. Paraffin hydrocarbons are quite desirable as Diesel fuels while the olefins and diolefins, aromatics and naphthenes do not have as desirable burning 20 characteristics. Next to ignition qualities of a fuel may be considered in their importance with reference to their burning characteristics the following properties: Viscosity, cleanliness, 25 boiling range, carbon residue and sulfur. In many types of Diesel engines, fuel is ignited by the heat of compression. In the engine design the maximum pressure is sought at which the fuel will ignite and it has been found that with many fuels there is a period of delay after the maximum 30 pressure has been reached before the fuel ignites. The longer the delay period, the more rapid is the rise in pressure and the greater is the amount of the final pressure. It is desirable therefore to minimize the duration of the delay period so as to have the fuel ignite almost 35 immediately after it has been raised to the pressure in the combustion chamber and thus to improve combustion and assure smoothness of engine operation.

It is common to increase the cetane value of 40 motor fuels to facilitate their combustion in a Diesel engine. Various ignition accelerators have been suggested. Among them are ethyl, propyl and butyl nitrates, alkyl nitrites, organic nitro compounds and nitro paraffins. Some of these 45 products have a distinct modifying value on the burning characteristics of fuel but none of them has proved entirely satisfactory. The nitrites tend to slightly raise the cetane number of a 50

motor fuel, but do it only when added in particularly large proportions. The lower alkyl nitrates which have been used tend to increase the cetane value of motor fuels, but this increase is peculiar in that a small amount of the alkyl nitrates give the maximum raise in cetane value and then additional amounts of the alkyl nitrates tend to decrease the cetane value. Furthermore these lower alkyl nitrates are explosive having low boiling point and flash point ranges and present a strong fire hazard. They also fail to improve startability sufficiently. It has been found, furthermore, that the lower alkyl nitrates are not completely soluble in hydrocarbon motor fuels and therefore it is necessary to use a blending agent in order to get them into solution in the motor fuels. Due to the low solubility of the compounds there is a tendency for the highly volatile low boiling alkyl nitrates to come out of solution and the presence of these vapors in the fuel tanks is a dangerous fire hazard, as well as being very explosive.

One of the features of this invention is to provide an improved method of operating an internal combustion engine and particularly a compression ignition engine by burning the fuel therein in the presence of amyl nitrates which act to lower the ignition temperature and to increase the rate of flame propagation.

In accordance with the present invention it has been found that most of the amyl nitrates and their mixtures have none of the defects inherent in other accelerators and give a comparatively large increase in the cetane value of hydrocarbon motor fuels. Amyl nitrates are more effective as ignition accelerators than lower alkyl nitrates. Of the eight isomers of amyl nitrates the normal primary amyl nitrate appears to have the most marked effect on the cetane value of hydrocarbon motor fuels. Other amyl nitrates having a marked effect are the secondary butyl carbinitrile the primary iso-amyl nitrate and the normal and the symmetric secondary amyl nitrates. These compounds are plentiful and comparatively cheap to manufacture. The approximate ranges of boiling points of amyl nitrates are as follows: primary normal amyl nitrate boiling points 152-156° C., secondary butyl carbinitrile boiling points 148-152° C., primary iso-amyl nitrate boiling points 146-148° C., mixed primary amyl nitrates boiling points 146-156° C., mixed secondary amyl nitrates boiling points 136-145° C., tertiary amyl nitrate boiling points 23-27° C. at 4/5 mm.

These amyl nitrates which properly may be called pentyl nitrates are manufactured from corresponding alcohols derived from natural gas or petroleum products and have the following molecular formulae:

- 60 1. Normal primary amyl nitrate or pentyl nitrate-1, or normal butyl carbinitrile-----  $\text{CH}_3\text{CH}_2\text{CH}_2\text{CH}_2\text{CH}_2\text{NO}_3$
- 65 2. Primary iso-amyl nitrate, or iso-amyl nitrate, or iso-butyl carbinitrile-----  $(\text{CH}_3)_2\text{CH}.\text{CH}_2\text{CH}_2\text{NO}_3$
- 70 3. Secondary butyl carbinitrile, a primary amyl nitrate-----  $\text{CH}_3.\text{CH}(\text{C}_2\text{H}_5).\text{CH}_2\text{NO}_3$
- 75 4. Methylpropyl carbinitrile or pentyl nitrate-2, or a secondary normal amyl nitrate-----  $\text{CH}_3.\text{CH}_2.\text{CH}_2.\text{CHNO}_3.\text{CH}_3$
5. Methyl-isopropyl carbinitrile, or a secondary iso-amyl nitrate-----  $(\text{CH}_3)_2\text{CH}.\text{CHNO}_3.\text{CH}_3$

6. Diethyl carbinitrile or pentyl nitrate-3, or a secondary amyl nitrate-----  $\text{C}_2\text{H}_5.\text{CHNO}_3.\text{C}_2\text{H}_5$
7. Dimethyl ethyl carbinitrile or tertiary amyl nitrate-----  $(\text{CH}_3)_2\text{C}.\text{CHNO}_3.\text{C}_2\text{H}_5$

The first three nitrates mentioned above are primary nitrates, the next three are secondary and the seventh isomer is a tertiary nitrate. Although all seven of these nitrates possess ignition accelerating properties, the effectiveness of each isomer greatly differs from one another. They also lower the temperatures of the ignition of Diesel engine fuels. The most effective are the primary amyl nitrates. The secondary, such as the diethyl carbinitrile and methyl propyl carbinitrile are also quite effective as agents for improving Diesel engine fuels, but are less effective than primary amyl nitrates. When the nitrates are made from mixed amyl alcohols derived from pentanes or from unsaturated petroleum hydrocarbons, such as for instance, amylenes or pentenes, we generally secure a mixture. In the first case such mixture is composed largely of primary nitrates and in the latter case a mixture is composed largely of the secondary nitrates. It has been found that these mixtures are very effective as agents for improving Diesel fuels and are technically and commercially practical for use in Diesel fuels.

It has been found that the increase in cetane value is substantially directly proportional to the percentage of amyl nitrates in the fuel. Furthermore the cetane value tends to increase along an almost straight line curve until more than 10 percent by volume of the amyl nitrates has been used in modifying the fuel.

It has been found that the amyl nitrates are substantially completely directly soluble in most hydrocarbon distillates in all proportions, do not require the use of blending agents and are non-corrosive.

The above isomeric compounds of the group of  $\text{C}_5\text{H}_{11}\text{ONO}_2$  were produced and tested individually, and in various mixtures with each other, in numerous Diesel fuels of various origins. The tests were made in standard Diesel testing engines using several known test methods and in several multi-cylinder compression ignition high speed service engines to determine their properties and effects and also the practicability for use.

The tests have developed that the members of the group  $\text{C}_5\text{H}_{11}\text{ONO}_2$  are neither equivalent in their effectiveness as ignition accelerators nor equivalent in their other properties. It has been found that the normal primary amyl nitrate is highly superior to the primary iso-amyl nitrate and to other amyl nitrates in its effectiveness as an ignition accelerator and in other valuable properties. It has also been found that the tertiary amyl nitrate is relatively effective as an ignition accelerator only when freshly made but after aging its effectiveness rapidly decreases until it becomes nil.

I have found that the effectiveness of Diesel fuel ignition accelerators such as mono- and poly-alkyl nitrates in general and amyl nitrates in particular and of peroxides of fatty acid anhydrides and the peroxides of ketones can be greatly increased by lowering the sulfur content in Diesel fuels. It appears that sulfur and the various sulphocompounds which are generally present in Diesel fuels affect unfavorably the catalytic activity of Diesel "dopes" by poisoning it or partly destroying it and thus they impair

their effectiveness as Diesel fuel ignition accelerators in engines. I have found that by removal of substantially all or of a larger part of sulfur and its compounds, i. e. by decreasing the sulfur content in a Diesel fuel the effectiveness of Diesel "dopes" and especially of amyl nitrates is increased so greatly that the cost of adding ignition accelerators to low-cetane number compression ignition fuels is minimized.

10 The following examples may be cited with reference to the properties of amyl nitrates:

|    | Fuel tested                                                                                          | Cetane number | Improvement |
|----|------------------------------------------------------------------------------------------------------|---------------|-------------|
| 15 | Base fuel, a Mid-Continent gas oil                                                                   | 50            | -----       |
|    | Base fuel plus 2% pentyl nitrates (mixed (70% primary and (30% secondary and tertiary amyl nitrates) | 67            | 17          |
|    | Base fuel plus 2% iso-amyl nitrate                                                                   | 68            | 18          |
| 20 | Base fuel plus 2% mixed primary amyl nitrates                                                        | 70            | 20          |
|    | Base fuel plus 2% normal primary amyl nitrate                                                        | 72            | 22          |

25 The addition of 2% of various amyl nitrates to the above Diesel fuel shows a substantial difference in their effectiveness as ignition accelerators. This difference increases when larger percentages of amyl nitrates are added to the base fuel. This test indicates that with 2% addition the normal primary amyl nitrate is about 30% more effective than a mixture of primary and secondary amyl nitrates. It is also by over 22% more effective than the primary iso-amyl nitrate and is about 10% more effective than mixed primary amyl nitrates. Pentyl nitrates comprised a mixture of about 70% primary (approximately 20% normal, 25% secondary butyl carbinitrate, 25% iso-amyl) and of about 30% secondary amyl nitrates (normal and diethyl carbinitrate). Mixed primary amyl nitrates comprised approximately 30% normal amyl nitrate, 55% secondary butyl carbinitrate and 15% iso-amyl nitrate.

30 In tests with other fuels, where the primary iso-amyl nitrate was added in larger percentages it proved to be by almost 14% less effective than 45 the above described mixture of primary and secondary amyl nitrates.

35 In order to establish the improvement of fuels in starting ability and in combustion the following tests were made:

|    | Sample                                           | O. C. R. critical compression ratio | Cetane number C. C. R. method | Cetane number ignition delay method |
|----|--------------------------------------------------|-------------------------------------|-------------------------------|-------------------------------------|
| 50 | Factory fuel                                     | 7.55                                | 65                            | 49                                  |
| 55 | Factory fuel plus 2% mixed primary amyl nitrates | 7.02                                | 78                            | 67                                  |
|    | Factory fuel plus 4% mixed primary amyl nitrates | 6.88                                | 83                            | 77                                  |

60 When larger percentages of nitrates were added the C. C. R. was reduced to as low as 5.03 and cetane value was increased to 100+ by both methods. It was evident from above that mixed amyl nitrates not only greatly improve combustion characteristics of Diesel fuels in compression-ignition engines but also greatly facilitate the starting. The ethyl nitrate and other lower alkyl nitrates however are lacking the property 65 of substantially improving the starting.

70 The following examples show how sulfur and sulfo-compounds content in Diesel fuels affects or influences the effectiveness of amyl nitrates as ignition accelerators in compression ignition engines.

| Fuel tested                                                                               | Total sulfur percent | Ignition delay cetane number | Improvements (in cetane) |
|-------------------------------------------------------------------------------------------|----------------------|------------------------------|--------------------------|
| High cetane ("Shell") secondary reference fuel (a straight run gas oil)                   | 0.34                 | 74                           | -----                    |
| High cetane "Shell"+1% mixed primary amyl nitrates                                        | 0.34                 | 84                           | 10                       |
| High cetane "Shell"+2% mixed primary amyl nitrates                                        | 0.34                 | 92                           | 18                       |
| Moderately high cetane fuel (a straight run gas oil)                                      | 0.074                | 52.5                         | -----                    |
| Moderately high cetane fuel +0.5% mixed primary and secondary amyl nitrates               | 0.074                | 65                           | 12.5                     |
| Moderately high cetane fuel +0.75% mixed primary and secondary nitrates                   | 0.074                | 72.4                         | 19.9                     |
| Moderately high cetane fuel +1% mixed primary and secondary amyl nitrates                 | 0.074                | 79.5                         | 27                       |
| Low cetane pressure still recycle gas oil (a cracked gas oil)                             | 0.26                 | 37.5                         | -----                    |
| Low cetane pressure still recycle gas oil +1% mixed (primary and secondary) amyl nitrates | 0.26                 | 48                           | 10.5                     |
| Low cetane pressure still recycle gas oil +2% amyl nitrates                               | 0.26                 | 50.6                         | 22.1                     |

25 No sulfur or sulfo-compounds were added or removed from the above Diesel fuels. The effectiveness of mixed amyl nitrates is decidedly greater with the diminishing of sulfur content in the above fuels. The ignition quality of natural Diesel fuels, that is a Diesel fuel distilled directly from a crude oil and which does not contain ignition accelerators, apparently does not change with either an increase or a decrease in the total sulfur content of the fuel. When, however, a given quantity of ignition accelerator is added to the fuel the ignition quality is appreciably better in the case of the fuel with the low sulfur content and the extent of the difference in the ignition quality in favor of the low sulfur content becomes even more marked when a desulfurization treatment is applied.

30 In the following examples the total sulfur content of a Diesel fuel was reduced from 0.156% to 0.109% and the effect of various concentrations of the primary iso-amyl nitrate in the fuel was determined before and after desulfurizing of the fuel to verify the improvement of its ignition quality in Diesel engine. The removal of this small quantity of 0.047% of sulfur content (which acted as a catalytic "poisoner") has resulted in a decided increase (by approximately 50% 45) in the effectiveness of the ignition accelerator in the fuels.

| Fuel                                                               | Total sulfur content | Ignition delay cetane No. | Improvements |
|--------------------------------------------------------------------|----------------------|---------------------------|--------------|
| Original fuel, (pressure still recycle gas oil), a cracked gas oil | Percent              |                           |              |
| Original fuel +0.5% iso-amyl nitrate                               | 0.156                | 38.5                      | 60           |
| Original fuel +1% iso-amyl nitrate                                 | 0.156                | 46.0                      | 7.5          |
| Original fuel +1.5% iso-amyl nitrate                               | 0.156                | 50.0                      | 11.5         |
| Desulfurized fuel (pressure still recycle gas oil)                 | 0.109                | 54.3                      | 15.8         |
| Desulfurized fuel +0.5% iso-amyl nitrate                           | 0.109                | 38.5                      | 65           |
| Desulfurized fuel +1% iso-amyl nitrate                             | 0.109                | 49.5                      | 11           |
| Desulfurized fuel +1.5% iso-amyl nitrate                           | 0.109                | 56.3                      | 17.8         |
| Desulfurized fuel +2% iso-amyl nitrate                             | 0.109                | 60.5                      | 22.0         |
| Desulfurized fuel +2.5% iso-amyl nitrate                           | 0.109                | 65.0                      | 26.5         |

75 It is apparent that sulfur and sulfo-compounds which are present in Diesel fuels tend to decrease the effectiveness of the ignition acceler-

erative property of amyl nitrates and therefore their removal is desirable, when amyl nitrates are used.

The above tests show that when the sulfur content of the hydrocarbon fuel is 0.05% by weight or less the effectiveness of the primary amyl nitrates for ignition acceleration and increasing the cetane number is more than double its effectiveness when the sulfur content is above 0.25%.

The preferred form of the invention having been thus described what is claimed as new is:

1. A liquid fuel for compression ignition engines comprising a high boiling petroleum hydrocarbon distillate of the gas oil type having dissolved therein less than ten percent by volume but sufficient to substantially increase the ignition acceleration of the fuel, of a pentyl nitrate selected from the group consisting of normal butyl carbinitrate, secondary butyl carbinitrate, methylpropyl carbinitrate, and diethyl carbinitrate.

2. A liquid fuel of the type defined in claim 1 wherein the pentyl nitrate may consist of a mixture of two or more nitrates of the defined group and wherein isobutyl carbinitrate may be mixed with one or more of the carbinitrates of the defined group.

3. A liquid fuel of the type defined in claim 1 wherein the petroleum distillate is a cracked petroleum distillate containing paraffinic, olefinic and other unsaturated hydrocarbons.

4. A liquid fuel of the type defined in claim 1 wherein the petroleum distillate is a cracked pe-

roleum distillate containing paraffinic, olefinic and other unsaturated hydrocarbons.

5. A liquid fuel of the type defined in claim 1 in which the petroleum distillate is a mixture of straight-run and cracked petroleum distillates containing olefinic, paraffinic and other unsaturated hydrocarbons.

6. A liquid fuel of the type defined in claim 1 wherein the hydrocarbon distillate is refined to reduce the sulfur content to less than .25 percent by weight of the distillate prior to addition of the nitrate to the distillate.

7. A process of enhancing the cetane susceptibility of high sulfur Diesel oils comprising hydrocarbon distillates of the gas oil type comprising refining the distillate to reduce the sulfur content to less than .25 percent by weight of the distillate and dissolving in the distillate a pentyl nitrate selected from the group consisting of normal butyl carbinitrate, secondary butyl carbinitrate, methylpropyl carbinitrate and diethyl carbinitrate.

8. A process of enhancing the cetane susceptibility of high sulfur Diesel oil comprising hydrocarbon distillates of the gas oil type comprising refining the distillate to reduce the sulfur content to less than .25 percent by weight of the distillate and dissolving a mixture of two or more pentyl nitrates in the distillate selected from the group consisting of normal butyl carbinitrate, secondary butyl carbinitrate, methylpropyl carbinitrate and diethyl carbinitrate and wherein isobutyl carbinitrate may be mixed with one or more of the nitrates of said group.

EUPHIME V. BERESLAVSKY. 35